

# UNITED STATES PATENT OFFICE.

HUGH S. COOPER, OF CLEVELAND, OHIO, ASSIGNOR TO THE ELECTRO METALS PRODUCTS COMPANY, OF CLEVELAND, OHIO.

## METAL ALLOY.

1,248,621.

Specification of Letters Patent. Patented Dec. 4, 1917.

No Drawing. Application filed January 21, 1916, Serial No. 73,332. Renewed October 8, 1917. Serial No. 195,458.

*To all whom it may concern:*

Be it known that I, HUGH S. COOPER, a citizen of the United States, residing at Cleveland, in the county of Cuyahoga and State of Ohio, have invented certain new and useful Improvements in Metal Alloys, of which the following is a specification.

This invention relates to an improvement in metal alloys, the object being to provide 10 a new and useful substitute for platinum for use in the electrical art. Platinum is used extensively for contact points in induction coils, magnetos, master vibrators, and high-frequency apparatus, and a practical 15 commercial substitute therefor must possess substantially the same hard and wearing properties, high-melting point electrical conductivity, ductility and malleability, and be non-oxidizing. I have dis- 20 covered that these requirements are met by alloying gold and silver in substantially equal proportions with a small percentage 25 of another metal adapted to harden and raise the melting point thereof. The metals 30 which may be added for this purpose may consist of osmium, niobium, rhodium, ruthenium, palladium, cobalt, molybdenum, tantalum, chromium, tungsten, thorium, titanium, vanadium, zirconium, or a combination 35 of these metals. Osmium is mentioned first as is preferred as about four per cent. of this metal in the alloy produces a fine hard metal which does not oxidize on the surface when used as an electrical contact. Specifically stated, an alloy consisting 40 of four per cent. of osmium, forty-eight per cent. of silver, and forty-eight per cent. of gold, is characterized by a high melting point, great hardness, its malleability and ductility so as to be easily worked, electrical conductivity similar to platinum, and by its low cost compared with platinum. The electrical conductivity of silver is rated at about 100, and gold 72, but I have dis-

covered that a combination of gold and silver in approximately equal proportions produces an alloy with an electrical conductivity of only about 15, or about one point less than platinum. Where the proportions of gold or silver vary from the foregoing by 50 an increase or decrease of five per cent. or more, the alloy is not especially suited for use as a contact for a magneto as the arc at the point of contact increases to such an extent that a regular series of sparks can 55 not be obtained.

The production of my improved alloy takes place preferably in an electric furnace and in an atmosphere free from oxidizing gases, and care must be exercised to have 60 the metals free from impurities such as copper, silicon, etc., as these tend to oxidize, thus making the product useless for electrical purposes.

What I claim is:

1. A metal alloy consisting of gold, silver and osmium having a high melting point and great hardness and possessing ductile and malleable properties and an electrical conductivity similar to platinum. 65

2. A metal alloy consisting of gold and silver in approximately equal proportions and a relatively small percentage of osmium. 70

3. A metal alloy consisting of gold and silver with the addition of approximately 75 four per cent. of osmium.

4. An electrical contact member made of an alloy composed in a preponderating degree of gold and silver and a relatively small proportion of osmium adapted to 80 harden the metal and raise the melting point thereof.

In testimony whereof I affix my signature in presence of two witnesses.

HUGH S. COOPER.

Witnesses:

R. B. MOSER,  
GEO. E. KRICKER.